# EUROPEAN PATENT SPECIFICATION

(11) **EP 0 484 542 B1**
(45) Date of publication and mention of the grant of the patent: **15.11.1995**
(21) Application number: 91908465.7
(22) Date of filing: 23.04.1991
(51) Int. Cl.: C10M 169/04, C10M 173/02

(54) **LUBRICANT COMPOSITION FOR METAL WORKING**
SCHMIERSTOFFZUSAMMENSETZUNG FÜR DIE METALLBEARBEITUNG
COMPOSITION LUBRIFIANTE POUR LA TRANSFORMATION DES METAUX

(30) Priority: 14.05.1990 JP 121361/90
(43) Date of publication of application: 13.05.1992
(73) Proprietor: IDEMITSU KOSAN COMPANY LIMITED, Tokyo 100 (JP)
(72) Inventor: KOYAMA, Saburo, Idemitsu Kosan Co., Ltd., Ichihara-shi, Chiba-ken 299-01 (JP); TOMARI, Yasunori, Idemitsu Kosan Co., Ltd., Ichihara-shi, Chiba-ken 299-01 (JP); SHIDO, Seiichi, Idemitsu Kosan Co., Ltd., Ichihara-shi, Chiba-ken 299-01 (JP); SAITO, Toshio, Idemitsu Kosan Co., Ltd., Ichihari-shi, Chiba-ken 299-01 (JP)
(74) Representative: Türk, Gille, Hrabal, Leifert
(86) International application number: JP9100534
(87) International publication number: WO9118074

(56) References cited:
- EP-A- 0 048 216
- EP-A- 0 369 320
- GB-A- 964 268
- JP-A- 0 284 495
- JP-A- 1 153 794
- JP-A- 1 282 297
- JP-A-63 202 697
- US-A- 3 288 715
- US-A- 3 536 622

## Description

### Technical Field

The present invention relates to a lubricating oil composition for metal working, particularly to a lubricating oil composition which comprises a specific type of straight chain olefin, alcohol and the like, and which has excellent detergency (removability) of abrasion dust produced in metal working of aluminum and aluminum alloy.

### Background Art

Generally, when straight chain-α-olefin is used as a lubricant in metal working such as plastic working (rolling or drawing), cutting, and grinding, working dust (abrasion dust) is adhered to the surface of a worked material after the working is finished. This results in deterioration of quality of a worked product and has unfavorable influence on the following working process.

For example, when an aluminum plate is rolled with the straight chain-α-olefin, aluminum abrasion dust is adhered to a rolled plate. If the rolled plate is annealed without removing such dust, annealing irregularity occurs very frequently. In case an aluminum foil is rolled by the use of the straight chain-α-olefin, there is a fear that pinholes are made on the aluminum foil because of the presence of abrasion dust. Likewise, abrasion dust is adhered to a worked material in cutting and grinding processes to cause various troubles.

### Disclosure of the Invention

In view of the above, the present inventors have earnestly pursued the studies in order to develop a lubricating oil for metal working which has excellent removability (detergency) of abrasion dust produced in metal working such as plastic working, cutting, and grinding performed on various kinds of metal such as aluminum, steel and brass, and alloys thereof, which is excellent in workability and capable of finishing the surface of a worked material in an excellent condition.

As a result, it has been found out that the above-mentioned object is accomplished when a lubricating oil composition for metal working consisting essentially of (a), (b) and (c) is used ; (a), (b) and (c) being defined as follows :
(a) a base oil which contains as an essential component at least 3% by weight of a straight chain olefin having 6 to 40 carbon atoms in admixture with at most 97% by weight of a mineral oil and/or a synthetic oil; the percent by weight is based on the weight of the base oil;
(b) at least one component selected from 0.05 to 50% by weight of a branched chain saturated or unsaturated aliphatic alcohol having 6 to 40 carbon atoms or straight chain saturated or unsaturated aliphatic alcohol having 6 to 20 carbon atoms and 0.05 to 1.0 % by weight of a straight/branched chain saturated/unsaturated fatty acid having 6 to 40 carbon atoms, based on the total amount of the composition; and
(c) not less than 0.1 % by weight based on the total amount of the composition of at least one compound selected from the group consisting of a phenolic compound represented by the following general formula (II) or (III): wherein each of R⁴ and R⁵ denotes an alkyl group having 1 to 8 carbon atoms and each of R⁶ and R⁷ denotes a hydrogen atom or an alkyl group having 1 to 6 carbon atoms and an amine compound represented by the following general formula (IV) or (V): wherein each of R⁸ and R¹¹ denotes a hydrogen atom or an alkyl group having 1 to 10 carbon atoms each of R⁹ and R¹⁰ denotes an alkyl group having 1 to 20 carbon atoms and each of R¹² to R¹⁴ denotes a hydrogen atom or an alkyl group having 1 to 20 carbon atoms;
   water being excluded.

### Best Mode for Carrying out the Invention

In the composition according to the present invention, the straight chain olefin constituting the base oil of the component (a) has 6 to 40 carbon atoms as described above. The straight chain olefin with the carbon atoms of less than 6 is undesirable because of a low flash point. If the number of carbon atoms is more than 40, the practical use is difficult because of a solid state. Furthermore, there become difficult the mixing with and the dissolving in mineral oil, synthetic oil, and other additives. In addition, the straight chain olefin having more than 40 carbon atoms is not popular and is difficult to be available. Among many kinds of the straight chain olefin, the composition having one double bond in a molecule and 6 to 30 carbon atoms is preferable. In particular, α-olefin (namely, n-α-olefin) having 12 to 30 carbon atoms are most preferable.

Specifically, examples for the straight chain olefin may include 1-octene, 1-decene, 1-dodecene, 1-tetradecene, 1-hexadecene, 1-octadecene, 1-eicocene, or mixtures thereof. The straight chain olefin can be produced by various methods. For example, there may be used ethylene oligomer obtained by polymerization of ethylene in an ordinary method.

According to the present invention mineral oil and/or synthetic oil is used together with the straight chain olefin. Water is excluded. Mineral oil and synthetic oil to be added have usually a kinematic viscosity of 0.5 to 500 cSt at a temperature of 40 °C, preferably, 0.5 to 30 cSt. Various kinds of mineral oil can be used, for example, distillate oil obtained through atmospheric distillation of paraffinic crude oil, intermediate crude oil, or naphthenic crude oil, or through vacuum distillation of residual oil in atmospheric distillation. Alternatively, there may be used refined-oils obtained by refining the distillate oil in a usual method, such as solvent refining, hydrogenation refining, dewax treating, and clay treating. When such mineral oil is mixed with the above-mentioned straight chain olefin, the resultant lubricating oil has an improved oxidation stability.

As synthetic oil, there may be used various types of olefin other than the above-mentioned straight chain olefin (for example, branched chain olefin such as polybutene and polypropylene), and hydrogenated product of such olefin. In particular, polybutene having low molecular weight, polypropylene having low molecular weight, and α-olefin oligomer having 8 to 14 carbon atoms are preferable. When such synthetic oil is mixed with the above-mentioned straight chain olefin, the resultant lubricating oil emits less odor during its use so as to improve working environment. Further, degreasing ability on the surface of a worked product is improved.

The mineral oil or the synthetic oil is mixed with the above-mentioned straight chain olefin to constitute the base oil of the component (a), the amount of the straight chain olefin is at least 3% by weight, preferably 5 to 60% by weight, while the amount of the mineral oil and/or the synthetic oil is at most 97% by weight, preferably, 95 to 40% by weight.

Then, as the component (b) in the composition according to the present invention, there is used one member selected from the group consisting of alcohol and fatty acid, or a combination of both members.

As alcohol, various alcohols may be used, and among them, aliphatic alcohol is preferable. Branched chain saturated or unsaturated aliphatic alcohol having 6 to 40 carbon atoms (especially 8 to 30 carbon atoms), or straight chain saturated or unsaturated aliphatic alcohol having 6 to 20 carbon atoms (especially 8 to 18 carbon atoms) is more preferable. The alcohol having less than 6 carbon atoms is rapidly consumed due to evaporation or splashing during its use and thus is economically disadvantageous. Branched chain alcohol having more than 40 carbon atoms or straight chain alcohol having more than 20 carbon atoms is sometimes undesirable since it may be insoluble in the base oil of the component (a).

Examples for such alcohol may include octyl (2-ethylhexyl) alcohol, decyl alcohol, lauryl alcohol, myristyl alcohol, cetyl alcohol, stearyl alcohol, eicosyl alcohol, oleyl alcohol, isostearyl alcohol, oxoalcohol, and the like. The amount of the alcohol is not limited, but it is suitable to use 0.05 to 50% by weight, preferably, 0.1 to 20% by weight, based on total amount of the composition.

As fatty acid, there are used straight/branched chain saturated/unsaturated fatty acid having 6 to 40 carbon atoms (preferably 8 to 20 carbon atoms). There is a risk that fatty acid having less than 6 carbon atoms are rapidly consumed due to evaporation or splashing during its use, while fatty acid having more than 40 carbon atoms is sometimes insoluble in the base oil of the component (a). Examples for such fatty acid may include caprylic acid, capric acid, lauric acid, myristic acid, palmitic acid, stearic acid, arachic acid, behenic acid, isostearic acid, undecylenic acid, oleic acid, linoleic acid, linolenic acid, arachidonic acid, and the like. The amount of fatty acid is 0.05 to 1.0% by weight, based on the total amount of the composition. If the amount of fatty acid exceeds 1.0% by weight, the anti-stain ability in annealing is unfavorably deteriorated.

As described, the composition according to the present invention comprises the above-mentioned components (a), (b) and (c) comprising at least one compound selected from the group consisting of phenolic compounds and amine compounds.

The phenolic compound represented by the following general formula (II) or (III) is used.
(In the formula, each of R⁴ and R⁵ denotes an alkyl group having 1 to 8 carbon atoms, and each of R⁶ and R⁷ denotes a hydrogen atom or an alkyl group having 1 to 6 carbon atoms.) Specifically, 2,6-di-tert-butyl-4-metylphenol (DBPC), 2,6-di-tert-butyl-4-ethylphenol, 2,2'-methylenebis (4-methyl-6-tert-butylphenol), 2,2'-methylenebis (4-ethyl-6-tert-butylphenol), and the like are preferable.

As amine compounds, it is suitable to employ usually the compounds represented by the following general formula (IV) or (V):
(In the formula, each of R⁸ and R¹¹ denotes a hydrogen atom or an alkyl group having 1 to 10 carbon atoms, each of R⁹ and R¹⁰ denotes an alkyl group having 1 to 20 carbon atoms, and each of R¹² to R¹⁴ denotes a hydrogen atom or an alkyl group having 1 to 20 carbon atoms.)

Specifically, di-p-octyldiphenylamine, di-p-butyldiphenylamine, di-p-nonyldiphenylamine, phenyl-α-naphthylamine, phenyl-β-naphtylamine, and the like are preferable.

The amount of the component (c) is preferably not less than 0.1% by weight, more preferably 0.1 to 2.0% by weight, based on the total amount of the composition.

If desired, a suitable amount of an oiliness agent, an extreme-pressure agent, a rust inhibitor, a corrosion inhibitor, a defoaming agent, or the like may be blended with the composition according to the present invention.

### Examples

Then, more detailed description will be made regarding the present invention with reference to examples and comparative examples.

### Examples 1 to 5 and Comparative Examples 1 to 10

The following rolling test was carried out by the use of lubricating oil for rolling which has the composition shown in Table 1.

### Rolling Test (Aluminum Plate Rolling)

A JIS A 5052 H16 aluminum plate (a coiled plate having a thickness of 1.2 mm and a width of 60 mm) was prepared as a material to be rolled. With each lubricating oil for rolling, the plate was rolled by a four-stage rolling mill having a work roll diameter of 135 mm at a rolling speed of 100 m/min. under forward tensions of 170 kgf and 400 kgf. The rolling process was carried out in such a manner that the reduction was stepwise increased per 20 m length during one pass as 50.0→ 54.2 → 58.3 → 60.8 → 63.3 → 65.8 → 68.3 (%). As to the plate having a thickness of 0.38 mm (a draft of 68.3 %) after the rolling process (after seven passes), the rolling load was measured. Abrasion dust detergency and anti-stain ability were evaluated by the following methods.

### (a) Evaluation Method for Abrasion Dust Detergency

### (Tape Test Method)

A cellophane tape was stuck onto the surface of the aluminum plate after rolling so as to pick up abrasion dust adhering thereto. Then, the tape was applied on a white paper sheet to visually determine a degree of contamination by abrasion dust. Thus, the detergency for abrasion dust adhering to the surface of the aluminum plate was evaluated. The results thus obtained are shown in Table 1.

### (b) Evaluation Method for Anti-stain Ability in Annealing

The aluminum plate after rolling was cut into piece having a short length of 10 cm. The stack of several tens of the cut pieces were fixed by a thick steel plate and annealed in a small-size annealing furnace.

The heating process in the annealing furnace comprises the step of: heating in an air atmosphere with a temperature rising rate of 5 °C/min. until the temperature reaches 330 °C; holding for 30 minutes; and cooling. After completion of the heating process, a degree of occurrence of annealing stains on the annealed plate was visually determined. Thus, the anti-stain ability was evaluated. The results are shown in Table 1.

### Comparative Examples 11 to 14

The following cutting test was carried out by the use of lubricating oil for cutting which has the composition shown in Table 2.

### Cutting Test (Cutting for End Face of Cylinder)

A cylindrical aluminum alloy material (AC-4A-T6) having a diameter of 80 mm was prepared as a material to be cut. The aluminum alloy material was cut to form an end face by the use of a cutting tool (cemented carbide P20) under the cutting condition that a cutting depth (t) is 1 mm and a feed rate (f) is 0.1 mm/revolution.

After the cutting, the surface roughness (R ₘₐₓ) of the cut end face was measured while the surface thereof was observed. The results are shown in Table 2.

### Industrial Applicability

As described above, by the use of a lubricating oil composition according to the present invention, abrasion dust detergency is improved in metal working (plastic working such as rolling, drawing, blanking, cold forging; cutting; and grinding) for various kinds of metals and alloys thereof while anti-stain ability in annealing of a worked material is improved.

Accordingly, a lubricating oil composition according to the present invention is widely and effectively used as a metal working oil in plastic working, cutting, or grinding of various kinds of metals and alloys such as aluminum, aluminum alloy, aluminum foil.

## Claims

1. A lubricating oil composition for metal working consisting essentially of
(a) a base oil which contains as an essential component at least 3% by weight of a straight chain olefin having 6 to 40 carbon atoms in admixture with at most 97% by weight of a mineral oil and/or a synthetic oil; the percent by weight is based on the weight of the base oil;
(b) at least one component selected from 0.05 to 50% by weight of a branched chain saturated or unsaturated aliphatic alcohol having 6 to 40 carbon atoms or straight chain saturated or unsaturated aliphatic alcohol having 6 to 20 carbon atoms and 0.05 to 1.0 % by weight of a straight/branched chain saturated/unsaturated fatty acid having 6 to 40 carbon atoms, based on the total amount of the composition; and
(c) not less than 0.1 % by weight based on the total amount of the composition of at least one compound selected from the group consisting of a phenolic compound represented by the following general formula (II) or (III): wherein each of R⁴ and R⁵ denotes an alkyl group having 1 to 8 carbon atoms and each of R⁶ and R⁷ denotes a hydrogen atom or an alkyl group having 1 to 6 carbon atoms and an amine compound represented by the following general formula (IV) or (V): wherein each of R⁸ and R¹¹ denotes a hydrogen atom or an alkyl group having 1 to 10 carbon atoms each of R⁹ and R¹⁰ denotes an alkyl group having 1 to 20 carbon atoms and each of R¹² to R¹⁴ denotes a hydrogen atom or an alkyl group having 1 to 20 carbon atoms;
water being excluded.

2. A lubricating oil composition for metal working according to claim 1 which contains further (d) at least one compound selected from the group consisting of oiliness agent, extreme-pressure agent, rust inhibitor, corrosion inhibitor and defoaming agent.

## Patentansprüche

1. Eine Schmierölzusammensetzung für die Metallbearbeitung, im wesentlichen bestehend aus
(a) einem Basisöl, das als wesentliche Komponente mindestens 3 Gew.-% eines geradkettigen Olefins mit 6 bis 40 Kohlenstoffatomen im Gemisch mit mindestens 97 Gew.-% eines Mineralöls und/oder eines synthetischen Öls enthält; die Gewichtsprozent sind bezogen auf das Gewicht des Basisöls;
(b) mindestens einer Komponente, ausgewählt aus 0,05 bis 50 Gew.-% eines verzweigtkettigen gesättigten oder ungesättigten aliphatischen Alkohols mit 6 bis 40 Kohlenstoffatomen oder eines geradkettigen gesättigten oder ungesättigten aliphatischen Alkohols mit 6 bis 20 Kohlenstoffatomen und 0,05 bis 1,0 Gew.-% einer geradkettigen/verzweigtkettigen gesättigten/ungesättigten Fettsäure mit 6 bis 40 Kohlenstoffatomen, bezogen auf die Gesamtmenge der Zusammensetzung; und
(c) nicht weniger als 0,1 Gew.-%, bezogen auf die Gesamtmenge der Zusammensetzung, mindestens einer Verbindung, ausgewählt aus der Gruppe, bestehend aus einer durch die folgende allgemeine Formel (II) oder (III) dargestellten phenolischen Verbindung: wobei R⁴ und R⁵ jeweils eine Alkylgruppe mit 1 bis 8 Kohlenstoffatomen und R⁶ und R⁷ jeweils ein Wasserstoffatom oder eine Alkylgruppe mit 1 bis 6 Kohlenstoffatomen bezeichnet und einer Aminverbindung, dargestellt durch die folgende allgemeine Formel (IV) oder (V) wobei jeweils R⁸ und R¹¹ ein Wasserstoffatom oder eine Alkylgruppe mit 1 bis 10 Kohlenstoffatomen bezeichnet und R⁹ und R¹⁰ jeweils eine Alkylgruppe mit 1 bis 20 Kohlenstoffatomen bezeichnet, und R¹² bis R¹⁴ jeweils ein Wasserstoffatom oder eine Alkylgruppe mit 1 bis 20 Kohlenstoffatomen bezeichnet;
wobei Wasser ausgeschlossen ist.

2. Eine Schmierölzusammensetzung für die Metallbearbeitung entsprechend Anspruch 1, die weiter (d) mindestens eine aus der aus Schmierfähigkeitsmittel, Extremdruckmittel, Rostinhibitor, Korrosionsinhibitor und Entschäumer bestehenden Gruppe ausgewählte Verbindung enthält.

## Revendications

1. Une composition d'huile lubrifiante pour le travail des métaux constituée essentiellement de
(a) une huile de base qui contient comme constituant essentiel au moins 3 % en poids d'une oléfine à chaîne droite ayant de 6 à 40 atomes de carbone en mélange avec au maximum 97 % en poids d'une huile minérale et/ou d'une huile synthétique ; les pourcentages en poids étant basés sur le poids de l'huile de base ;
(b) au moins un constituant choisi parmi 0,05 à 50 % en poids d'un alcool aliphatique saturé ou insaturé à chaîne ramifiée ayant 6 à 40 atomes de carbone ou d'un alcool aliphatique saturé ou insaturé à chaîne droite ayant 6 à 20 atomes de carbone et 0,05 à 1,0 % en poids d'un acide gras saturé ou insaturé à chaîne droite ou ramifiée ayant 6 à 40 atomes de carbone, par rapport à la quantité totale de la composition ; et
(c) pas moins de 0,1 % en poids, par rapport à la quantité totale de la composition, d'au moins un composé choisi dans le groupe constitué par un composé phénolique représenté par la formule générale (II) ou (III) suivante où chacun de R⁴ et R⁵ représente un groupe alcoyle ayant 1 à 8 atomes de carbone et chacun de R⁶ et R⁷ représente un atome d'hydrogène ou un groupe alcoyle ayant 1 à 6 atomes de carbone et un composé aminé représenté par la formule générale (IV) ou (V) suivante : où chacun de R⁸ et R¹¹ représente un atome d'hydrogène ou un groupe alcoyle ayant 1 à 10 atomes de carbone, chacun de R⁹ et R¹⁰ représente un groupe alcoyle ayant 1 à 20 atomes de carbone et chacun de R¹² à R¹⁴ représente un atome d'hydrogène ou un groupe alcoyle ayant 1 à 20 atomes de carbone ;
l'eau étant exclue.

2. Une composition d'huile lubrifiante pour le travail des métaux selon la revendication 1, qui contient en outre (d) au moins un composé choisi dans le groupe constitué par les agents d'onctuosité, les agents extrême-pression, les agents antirouille, les inhibiteurs de corrosion et les agents antimousse.
